

# UNITED STATES PATENT OFFICE

SIDNEY G. THOMAS, OF 3 QUEEN'S ROAD VILLAS, COUNTY OF SURREY,  
ENGLAND.

## BASIC PROCESS OF TREATING IRON IN THE MANUFACTURE OF BESSEMER STEEL.

**SPECIFICATION** forming part of Letters Patent No. 253,130, dated January 31, 1882.

Application filed November 8, 1879. Patented in England September 3, 1879, in Belgium October 15, 1879, and in France December 5, 1879.

*To all whom it may concern:*

Be it known that I, SIDNEY GILCHRIST THOMAS, of 3 Queen's Road Villas, in the county of Surrey, England, have invented a 5 certain Improvement in the Basic Process of Treating Iron in the Manufacture of Bessemer Steel, which process is fully described in the following specification.

In carrying out my process for the manufacture of Bessemer steel from phosphoretic pig-iron, as described in my Patent No. 217,495, dated July 15, 1879, in a basic-lined vessel, with a calcareous slag and an "after-blow," I have found that instead of adding to the dephosphorized and decarburized metal spiegel-eisen or ferro-manganese in the ordinary way, a greatly improved result in the economy of manganese, the reduction of the tendency of the spiegel to put back the phosphorus from the 10 into slag the steel, and freedom from red-shortness is obtained by proceeding as follows: To the decarburized and dephosphorized metal, at the termination of the after-blow, I add from three to seven per cent. of molten pure 15 pig-iron containing preferably less than 10 per cent. (one-tenth) of phosphorus and sulphur, and at least one per cent. of silicon and less than three per cent. thereof. I then immediately after add to the metal sufficient rich 20 spiegel or ferro-manganese to give the desired amount of manganese and carbon to the steel. I find for hard rail-steel six or seven per cent. of pure pig-iron containing about two per cent. of silicon, followed by five per cent. of 25 spiegel, with fifteen to seventeen per cent. of manganese, is a good proportion. The spiegel-eisen or ferro-manganese should also be molten, or, in the case of ferro-manganese, red-hot lumps may sometimes be used. By this 30 means I deoxidize the metal by the carbon and silicon of the pure pig-iron without wasting manganese, thus effecting a notable economy 35 of manganese, and I also reduce the tendency of the spiegel to put back phosphorus from the slag into the steel, and I produce a higher 40 quality of steel, entirely free from any tendency to red-shortness. This addition of pig-iron is only advantageous when using a calca-

reous slag and lining and an after-blow, as before described by me. 50

It is at present the practice to recarburize Bessemer refined metal made by the ordinary or acid process by adding to it a certain quantity of spiegel-eisen or of ferro-manganese. It has also been proposed to add to refined Bessemer metal a mixture of pure pig-iron and metallic manganese, and it has been proposed to add, in general terms, the additions which are necessary for manganese, and, if wished, also carbon and silicium. 55 60

It has further been proposed, in order to make sound castings from ordinary—that is, undephosphorized—Bessemer or Siemens steel, to add silicon to the metal, either by means of an addition of a special highly-silicious pig-iron, containing from five to ten per cent. of silicon, followed by ferro-manganese, or by an addition of a special compound of silicon, manganese, and iron, known as "silico-ferro-manganese." This addition is specially directed 70 to be made, and has always been made in such proportions as to leave from one-tenth to six-tenths of silicon in the steel, and, as I have before observed, the addition is always made either as a special compound of silicon, manganese, and iron, or a special highly-siliconized pig-iron—that is, a special pig-iron containing over five per cent. of silicon—the object always being to leave one-tenth per cent., or more, of silicon in the steel—a thing which 75 80 is, for my purpose, highly prejudicial.

Now, none of these methods, if applied to dephosphorized metal, answers the purpose I have in view—namely, the prevention of rephosphorization, the saving of manganese and iron, and the giving a very high quality of metal, eminently suited for rolling and forging without red-shortness; and I do not claim any of these processes, nor do I claim the use of silico ferro-manganese, or of a pig-iron containing over five per cent. of silicon, as an addition; but 85 90

What I claim as new, and constituting the subject of my present invention, is—

The herein-described improvement in the 95 process of treating iron, which consists in add-

ing to the refined metal which has been de-phosphorized in a basic-lined converter, with basic additions at the end of the after-blow, from three to seven per cent. of ordinary non-phosphoric pig-iron, preferably containing less than three per cent. of silicon, immediately followed by the addition of spiegeleisen or ferro-manganese, so as to recarburize the metal and prevent red-shortness, without rephosphor-

izing it, without wasting manganese, and without leaving so much as one-tenth per cent. of silicon in the metal, substantially in the manner and proportions herein described.

SIDNEY GILCHRIST THOMAS.

Witnesses:

PHILIP S. JUSTICE,  
ALLEN P. JONES.